

May 21, 1940.

G. G. MORENO

2,201,591

PHOTOGRAPHIC PROCESSING

Filed May 11, 1939



GABRIEL GARCIA MORENO  
INVENTOR

BY

*C. J. McRell*

ATTORNEY

## UNITED STATES PATENT OFFICE

2,201,591

## PHOTOGRAPHIC PROCESSING

Gabriel Garcia Moreno, Mixcoac, D. F., Mexico,  
assignor to CMC Corporation, New York, N. Y.,  
a corporation of Delaware

Application May 11, 1939, Serial No. 273,023

6 Claims. (Cl. 95—88)

The present invention relates to an improved method of photography whereby pictures of better quality and greater range of density variations may be obtained. It also relates to a method of processing any and all types of emulsions subsequent to exposure and prior to development whereby the latitude of the emulsion is greatly enhanced, its inertia very materially reduced, and the developability of the latent image very materially increased, so that in effect the sensitivity of the emulsion is increased to say 400% or 700% of its original value.

Moreover, the invention relates to means and reagents particularly adapted for use in such treatment, these reagents being hereinafter referred to as activating compounds. Although the present invention is applicable for use in all forms of photography, it appears to be particularly well adapted for use in motion picture work since the processing may be carried out rapidly and for this reason may be coordinated with the usual continuous developing processes used in motion picture film laboratories. Moreover, the use of the process gives rise to very material savings in time and money when used in motion picture work.

In motion picture photography, very intense illumination is employed, necessitating numerous electricians and sources of illumination and therefore by increasing the cost and rendering working conditions on the set or scene disagreeable. The present invention permits the use of from one-fourth to one-seventh of the light intensity ordinarily employed and in some instances good results are obtained with materially smaller intensities of light. The methods and means of this invention are therefore of considerable value in monochromatic and in color motion picture photography.

There are other instances where available light intensity is not sufficient for the production of good pictures by the ordinary methods. For example, in the background projection method (where a background picture is projected upon a screen and such projected image is then photographed in conjunction with actors) difficulties have been heretofore encountered. Newspaper photographers often desire to obtain photographs at night or in improperly illuminated areas. By means of the reagents hereafter described, any photographic emulsion carrying a latent image is capable of being treated so as to produce a good visible image even though the ordinary methods of development would not produce a good visible image.

An object of the present invention, therefore, is to provide a reagent containing activating materials and compounds, such reagent being adapted for use in the treatment of photographic emulsions containing latent images whereby the

latent image is rendered developable to such an extent that whereas ordinarily no image would be obtained, a fully graded, well defined and detailed image is now obtained in accordance with this invention.

The activating solutions of this invention are aqueous alkaline solutions containing meta-substituted amino derivatives of benzene and benzene ring amino hydroxyl compounds derived from benzene or naphthalene and having a substituting radical in the meta position or 1,3- relation to the amino or hydroxyl group. The action of these activating compounds is not well understood but such compounds tend to act as normal developers. Many developers are benzene ring compounds but developers are distinguishable from the activating compounds of this invention in that developers contain substituents in the para position and are capable of distinguishing between exposed and unexposed grains in an emulsion. Moreover, normal developers do not render visible latent images of the character which are rendered developable by the activating substances disclosed herein.

An object of the invention is to provide a method and means for treating photographic emulsions whereby better quality, greater range in tonal values and greater latitude are obtained.

Another object is to provide a method of treating photographic film whereby underexposed emulsions may be developed to form images having the required degree of contrast and definition.

Another object is to provide means for and methods of treating exposed films to increase their latitude and ability to reproducibly record a wider range of density gradations.

Still another object is to provide means for and methods of treating previously exposed photographic film whereby latent images which are not responsive to usual development are now made developable.

Other objects, advantages, uses and adaptations will become apparent to those skilled in the art from the following description.

As previously stated, the primary reagent to be employed in the performance of the inventions herein is an aqueous, alkaline solution containing an activating agent, such activating agent being any meta-substituted amino derivative of benzene or any benzene ring amino hydroxyl compound derived from benzene or naphthalene and having a substituting radical in the meta position or 1,3- relation to the amino or hydroxyl group. A large number of activating agents have been found satisfactory, among them meta-dihydroxy-benzene, meta-phenylene-diamine, meta-nitraniline, meta-toluidine, meta-toluene-diamine (2,4- diamino toluene), meta-cresol, meta-amino-phenol, 2,4- diamino-phenol-dihydrochloride, 2,4- diamino-anisole-dihydro-

chloride, etc. Each of the substances mentioned and embraced by the general group is capable of producing a certain maximum effect upon the latent image in the exposed photographic emulsion and this effect can be increased somewhat by combining two or more of the activating agents in the same bath or solution. The solution may contain from about 0.15% to 2.5% by weight of the meta compounds embraced by the group mentioned. Such solution may also contain a dispersing or solubilizing aid; for example, when a difficultly soluble activating compound is being employed, alcohol acetone or other water-miscible solvent may be used in the solution for the purpose of dispersing and solubilizing the activating compound.

The treating and activating solution should be alkaline and its alkalinity may be equivalent to that obtained by the use of about 0.3% to 1.0% of sodium hydroxide by weight. Small amounts of sodium hydroxide may therefore be present in the solution, although other alkali or alkaline salts and substances may be present such as, for example, any of the salts of strong bases and weak acids such as borax, sodium phosphate, sodium citrate and the like. Moreover, the solution may contain an antioxidant or stabilizing material such as sodium sulfite.

The concentration of the activating agents in the treating bath may be varied appreciably and the presence or absence of numerous ingredients will depend somewhat upon the conditions encountered and the manner in which the treating bath is to be employed. The following illustrative examples are typical:

|                          |          |       |
|--------------------------|----------|-------|
| Acetone                  | 25 cc.   | 1.1%  |
| Meta-cresol              | 15 cc.   | 0.7%  |
| Meta-toluene-diamine     | 10 gr.   | 0.5%  |
| Meta-nitraniline         | 1.25 gr. | 0.06% |
| Meta-resorcinol          | 10 gr.   | 0.5%  |
| Sodium sulfite           | 50 gr.   | 2.2%  |
| Potassium meta-bisulfite | 50 gr.   | 2.2%  |
| Water                    | 1 litre  | 92.7% |

It is to be understood that the above represents a treating solution of approximately the concentration used in treating the exposed film. Weaker solutions have been found very effective, as for example, those obtained by diluting the bath with another litre of water. Moreover, the solutions may be prepared in more concentrated form and then diluted shortly prior to use.

A solution of the specific character given hereinabove may be used with advantage by adding the same to a litre of water containing approximately 7 grams of sodium hydroxide, 90 grams of sodium sulfite and a very small quantity, say  $\frac{1}{2}$  gram, of potassium bromide.

Another typical treating solution may comprise the following:

|                        |          |
|------------------------|----------|
| Meta-dihydroxy-benzene | 1 gram   |
| Meta-toluidine         | 0.75 gr. |
| Meta-phenylene-diamine | 0.25 gr. |
| Meta-nitraniline       | 0.25 gr. |
| Acetone                | 5 cc.    |
| Sodium phosphate       | 15 gr.   |
| Water                  | 1000 cc. |

In some instances when a treating solution is being manufactured, the sequence in which the ingredients are incorporated in the solution influences the results obtained. For example, when m-dihydroxy-benzene is being employed, it is desirable to incorporate the stabilizer, such as sodium sulfite, in a water solution, then add the

activating agent, and finally render the solution alkaline by the addition of sodium phosphate, borax or the like.

The effect of a treatment of exposed but undeveloped film with a treating solution having the above composition is graphically shown on the appended drawing. The ordinates represent densities whereas the abscissa represent exposure or light intensity. The abscissa numbered from 1 to 20 are indications of exposure corresponding to those used on the sensitometric strips made on the machines approved and used by Eastman Kodak Company. Curve 10 shown on the appended drawing represents the characteristics of a standard Eastman Super X film whereas curve 11 depicts the characteristics of the same type of film which has been treated, after exposure and prior to development, with the activating agent solution described hereinabove.

Attention is particularly called to the fact that the length of the straight line portion of curve 11 is appreciably greater than the straight line portion of curve 10. For an exposure of 16, the ordinary development produces a density of 0.39 whereas for the same exposure the film treated in accordance with this process has an exposure of 0.90. From a contemplation of these two curves it will be quite evident that the inertia of the film is materially reduced and the latitude of the film very greatly increased. The graphs shown are for film developed to a gamma of 67.

The use of the solution described hereinabove in the treatment of film may involve several modifications. In one method, exposed photographic emulsion containing a latent image is subjected to the action of the activating agent solution, washed and then subjected to the action of a developing bath. The activating solution in such instances does not contain any developers. The film or emulsion, after being treated with the activating reagents and washed, may be dried before it is subjected to the action of the developer, although drying is not essential. The graphical illustration appended here-to illustrates this method of treatment. When this method is carried out, it will be found that the temperature at which the treating solution is applied does not materially affect the results and therefore temperatures from say about 50° F. to 90° F. may be used. Furthermore, the time of treatment or the time during which the activating solution is permitted to act on the film may vary within wide limits. Ordinarily, times of treatment ranging from 4 to 15 minutes are entirely satisfactory, although even shorter times may be used.

X-ray emulsions and extremely sensitive emulsions such as those employed by press photographers, are very effectively treated by adding a solution of activating agents of the character described hereinabove directly to a developing bath of any suitable type. The exposed film carrying an emulsion bearing a latent image can then be developed in the solution of the activating agents and developers and under these conditions the activating agents appear to act upon the latent image immediately prior to the development of the images with the production of negatives, or positives as the case may be, which show greater detail and less fog than is obtained by the use of the developer alone or by the sequential use of activating agents and developer. Ordinarily, from about 0.3 volume to 75

2.0 volumes of an activating solution of the character mentioned hereinbefore may be added to 1 volume of any commercial developing solution with very good results.

It will be found that usually the time necessary for development in the subsequent step can be materially reduced from that normally employed with the developer, assuming temperature and concentration conditions of the developing solution to be constant.

In addition to simple meta-substituted amino derivatives, the present invention contemplates the use of the secondary substitution products, such as meta-substituted diamino- or hydroxy-amino benzene derivatives, one or more amino groups of which may carry methyl or other alkyl groups as substituents on the nitrogen, the amino or hydroxyl groups of such compounds being in a 1,3- relationship to each other. Examples of such secondary substitution products which can be used successfully are: mono-methyl-meta-phenylene-diamine-dihydrochloride; 2,4- di-amino-anisole-dihydrochloride; meta-methyl-aminophenol; dimethyl-metaphenylene-diamine; etc. Since different photographic emulsions often exhibit minor differences in their reaction to the activating solutions and to different developers, the operator may wish to try a number of activating agents from the groups referred to before selecting those which produce results most agreeable to his taste.

This application is a continuation-in-part of Serial No. 140,626, filed May 4, 1937.

I claim:

1. In a process of treating exposed photographic emulsions containing a latent image, the steps of subjecting a photographic emulsion after exposure and prior to development to the action of an aqueous alkaline medium containing from about 0.2 to 4.0 grams of an activating agent from the group consisting of meta-phenylene-diamine, meta-nitraniline and meta-toluidine, per 1000 cc. of said medium, for a period of from 2 to 10 minutes and in the absence of a developer, then washing and drying the film, and then developing the film in a developer for a shorter time than that normally employed for such developer.

2. In a process of treating photographic emul-

sions containing a latent image, the steps of: subjecting a photographic film after exposure and prior to development to the action of an alkaline aqueous medium free from developers and containing an activating agent from the group consisting of meta-dihydroxy-benzene, meta-phenylene-diamine, meta-nitraniline and meta-toluidine, and then developing, washing and drying the film.

3. A process of the character defined in claim 10 2 in which the said aqueous medium contains from about 0.2 to 2.0 grams of activating agent per 1000 cc. of medium.

4. A solution for use in the treatment of photographic silver halide gelatin emulsions containing latent images, comprising: an aqueous alkaline solution containing from about 0.15% to 2.5% of an activating agent from the group consisting of meta substituted amino derivatives of benzene, having a substituting radical in the 20 meta position to the amino group, derivatives of 1-aminonaphthalene having a substitution radical in the 3 position, and derivatives of 2- amino-naphthalene having a substitution radical in the 4 position, said solution having an alkalinity 25 equivalent to between about 0.3% and 1.0% sodium hydroxide by weight.

5. A solution for use in the treatment of photographic silver halide gelatin emulsions containing latent images, comprising: an aqueous 30 alkaline solution containing from about 0.15% to 2.5% of an activating agent comprising a meta substituted amino derivative of benzene, having a substituting radical in the meta position to the amino group, said solution having an alkalinity 35 equivalent to between about 0.3% and 1.0% sodium hydroxide by weight.

6. A process of treating underexposed silver halide gelatin negatives containing latent images to properly develop the same, comprising: subjecting an underexposed photographic emulsion containing a latent image to the action of an aqueous alkaline medium containing from about 0.15% to 2.5% by weight of a meta substituted amino derivative of benzene having a substituting radical in the meta position to the amino group.

GABRIEL GARCIA MORENO.